

Jan. 13, 1931.

N. E. NEWMAN

1,789,111

STRUCTURAL SLAB OR PANEL

Filed Sept. 19, 1928



INVENTOR  
*Nathan E. Newman*

BY

*Wm. J. Jones*  
ATTORNEY

## UNITED STATES PATENT OFFICE

NATHAN E. NEWMAN, OF BRONXVILLE, NEW YORK

## STRUCTURAL SLAB OR PANEL

Application filed September 19, 1928. Serial No. 306,984.

My invention relates to the method of manufacturing slabs or panels which are essentially waterproof and fireproof, and upon one surface of which appears an exact imitation of marble or other patterns. The base material of which the slabs are formed is comminuted asbestos, preferably combined with a suitable binder, and primarily, because of the very reasonable cost of these materials, the finished product is adapted to a wide field of use, in fact, it may be economically employed any place in building construction as a substitute for real marble or other relatively expensive patterns, as ceramic tiling effects, etc.

The first, and by far the most important step concerned in my method is the preparation of the slab. It must be rendered thoroughly waterproof, and in producing this most essential characteristic it must not be lost sight of that whatever material is used to produce the waterproof quality must necessarily combine with or have an affinity for a filler, such as a lacquer. Otherwise, if the base material were attacked by moisture, all of the layers of coating subsequently applied would rapidly disintegrate and thereby render useless the very purpose of the slab. So, in this connection, it is not deemed amiss to amplify in a general way the manner in which I proceed. Firstly, the slab is dried for a considerable period of time. Then it is immersed in a bath of suitable waterproofing preparation, and one which will combine with a filler, such as a lacquer. The slab is permitted to remain in this bath until the waterproofing preparation has had an opportunity to penetrate the pores or interstices of the base material. After conducting a number of experiments I have discovered that vegetable oil, suitably thinned by the addition of naphtha, possesses all of these desirable qualities.

For a more specific explication of my invention, attention is invited to the accompanying drawings, in which the numeral 1 designates a slab constructed from fine asbestos and any desirable binder. This slab is first dried in an oven for a period of approximately 24 hours, after which it is im-

mersed in a bath comprising an admixture of vegetable oil and a thinner therefor, as naphtha. It is allowed to remain in this bath for about one and a half hours, during which time the liquid penetrates deeply into the slab from all sides and ends, effectively occluding the pores or interstices of the material. The slab is then withdrawn from the bath and the surplus liquid wiped off, whereupon the said slab is subjected to a further drying extending over a period of about 24 hours. After it has been allowed to cool the slab is put through a sanding machine which serves to eliminate any undulatory surfaces which may be present, and otherwise render it comparatively smooth. At this stage of the method very minute depressions remain in the slab but these depressions are filled by the next step which comprises the application of a coat of lacquer 2 while the slab is being fed between two or more rolls, commonly known as a "puttying machine". Thereupon the lacquer on the slab is allowed to dry for approximately 24 hours, and two more coats of lacquer 3 and 4 sprayed thereon, or otherwise suitably applied, and then dried for 24 hours, this operation producing what is known as a substantial "sanding surface". By again placing the slab in the sanding machine for a period of two or three minutes, the outer surface is rendered perfectly smooth, and it is only necessary to spray thereon another coat of lacquer 5 and allow it to dry for about an hour in order to produce a surface which is eminently suited to receive a pattern 6. This pattern may consist of reproducing by photogravure the exact brecciated or veined effect of marble, and may even include a diversity of tints and delicate colors which are diffused through marble in irregular patches. In any event, the pattern is transferred to the slab, and as a protective coating two additional applications of lacquer 7 and 8 are made and when these are dry the slab is placed in a polishing machine and very highly polished.

By the method as hereinbefore explained, I produce a slab or panel which perfectly

reproduces standard marble and all of its desirable qualities. It is water proof and fireproof—it will not crack nor warp—it is entirely sanitary, easily cleaned, and may be quickly attached to concrete or brick walls by the customary method of furring, or by using any suitable plastic compound.

I desire to reserve the right to effect such modification as may come fairly within the scope of the appended claims. For example, my method is not necessarily restricted to the inclusion of replicas of marble patterns. The slab or panel herein described may be employed as a foundation for other reproductions or designs.

What I claim is:

1. The herein described method of preparing an imitation marble slab or the like, comprising the steps of drying an asbestos slab, immersing it in a waterproofing bath, permitting it to dry, applying a filler, applying a coating of lacquer, rendering the lacquered surface smooth, transferring to said surface by photogravure process a facsimile marble pattern, applying a coating over the pattern, and highly polishing said coating.

2. The method of preparing a decorative slab in imitation of marble or the like, comprising drying an asbestos base layer, impregnating the base with waterproofing material, approximately smoothing a surface of the base, applying to said surface one or more coatings of a filler of character adapted to adhere to the base and water proofing content thereof, smoothing the filler surface, imprinting on the smooth surface a decorative design in imitation of natural marble or the like, and applying over the design a protective coating.

3. The method of preparing a decorative slab in imitation of marble or the like, comprising drying an asbestos base layer, impregnating the base with waterproofing material, approximately smoothing a surface of the base, applying to said surface one or more coatings of a filler of character adapted to adhere to the base and water proofing content thereof, smoothing the filler surface, spraying a thin coating of filling material on the smooth surface, imprinting on the smooth surface a decorative design in imitation of natural marble or the like, and applying over the design a protective coating.

4. The method of preparing a decorative slab in imitation of marble or the like, comprising thoroughly drying a base layer consisting of asbestos and a binder, impregnating the base with waterproofing material including a vegetable oil and a thinner, drying the base, approximately smoothing a surface of the base, applying to said surface one or more coatings of a filler of character adapted to adhere to the base and waterproofing content thereof, smoothing the filler surface, imprinting on the smooth surface a decorative

design in imitation of natural marble or the like, applying over the design a protective coating, and polishing the coating.

5. The method of preparing a decorative slab in imitation of marble or the like, comprising thoroughly drying a base layer consisting of asbestos and a binder, impregnating the base with waterproofing material including a vegetable oil and a thinner, drying the base, approximately smoothing a surface of the base, applying to said surface one or more coatings of a filler of character adapted to adhere to the base and waterproofing content thereof, smoothing the filler surface, spraying a thin coating of filling material on the smooth surface, imprinting on the smooth surface a decorative design in imitation of natural marble or the like, and applying over the design a protective coating.

6. As an article of manufacture, a decorative imitation marble slab comprising an asbestos base sheet treated with waterproofing material, a filler coating on a surface of the base, a decorative design, imitative of marble or the like imprinted on the filler coating, and a transparent protective coating on the design.

7. As an article of manufacture, a decorative imitation marble slab comprising an asbestos base sheet impregnated with waterproofing material, a filler coating on a smoothed surface of the base, a decorative design imitative of marble or the like imprinted on the filler coating, and a polished transparent protective coating on the design.

8. As an article of manufacture, a decorative imitation marble slab comprising a base sheet consisting of asbestos and a filler and impregnated with a vegetable oil, a filler coating of lacquer on a surface of the base, a decorative design imitative of marble or the like imprinted on the filler coating, and a polished transparent protective coating on the design.

Signed at New York city, in the county of New York, State of New York, this 21st day of August, 1928.

NATHAN E. NEWMAN.

115

120

95

120